# EUROPEAN PATENT SPECIFICATION

(11) **EP 2 944 709 B1**
(45) Date of publication and mention of the grant of the patent: **24.07.2019**
(21) Application number: 15460013.4
(22) Date of filing: 30.04.2015
(51) Int. Cl.: C25C 1/10, C25C 5/02

(54) **A METHOD FOR ELECTROWINNING OF METALLIC CHROMIUM FROM ACIDIC WASTE ELECTROLYTES**
VERFAHREN ZUR ELEKTROLYTISCHEN GEWINNUNG VON METALLISCHEM CHROM AUS SAUREN ABFALLELEKTROLYTEN
PROCÉDÉ D'EXTRACTION ÉLECTROLYTIQUE DE CHROME MÉTALLIQUE À PARTIR D'ÉLECTROLYTES D'EAUX USÉES ACIDES

(30) Priority: 07.05.2014 PL 40812914
(43) Date of publication of application: 18.11.2015
(73) Proprietor: Nycz, Ryszard, 38-524 Besko (PL)
(72) Inventor: Nycz, Ryszard, 38-524 Besko (PL)
(74) Representative: Bartula-Toch, Marta

(56) References cited:
- DE-C- 639 446
- US-A- 1 544 451
- US-A- 2 803 594
- US-A- 5 433 797

## Description

The subject of the invention is a method for electrowinning of metallic chromium from aqueous acidic waste solutions of complex composition.

Due to environmental concerns, in recent years most countries of the world have been changing rules and tightening requirements for all human activities in the scope of water, soil and air protection. At the same time, in the era of expansive human economy, the demand for metals, including heavy metals, has increased to such an extent that some of these resources are running out. A growing concern is also the deteriorating quality of ores mined worldwide, the decline in the quality of concentrates and metal yields, as well as the rising cost of metal production.

This situation makes it necessary to endeavour to increasingly recover raw materials, including chromium compounds from waste solutions.

Dangerous sewage containing highly toxic chromium originates mainly from tanneries, dyeworks, electroplating plants, chromium plants etc. Despite many studies on chromium recycling, the problem of its recovery, especially in metallic form, along with the simultaneous sewage treatment, remains unresolved. The technology of disposal of waste containing Cr(VI) uses almost exclusively a reduction method of Cr(VI) chromium ions to Cr(III), involving the precipitation of insoluble chromium hydroxide, which is then stored at a solid waste landfill.

The patent application P. 381 326 discloses a method for comprehensive management of tannery waste, including chromium solid waste, combined with processing of sewage sludge, including sludge containing chromium (III). This method consists in the purification of waste and sludge from chromium during the initial stages of the closed process, both by leaching chromium (III) with working solutions containing at least one base salt, one extractant and one pH regulator, and by liquid/liquid extraction removal using a catalyst of phase transfer of chromium (III) and other, previously complexed, trivalent metals from waste water into the organic phase. Purified waste and sludge and inorganic compounds generated in the course of their treatment are processed into valuable products during subsequent process stages. The method results in recovering untanned hide collagen with intact fibrous structure, chromium compounds and other inorganic salts which were previously pollutants of chromium sewage sludge.

U.S. patent US4948476 discloses a method for recovering chromium from industrial sludge and a device for applying the method. Electrolysis of the solution containing chromium ions is carried out in a system composed of at least one anode, one cathode and an anion exchange membrane which are connected to a DC power source. The membrane is made of poly(p-trimethylaminomethyl)styrene, poly(p-dimethylaminomethyl)styrene or (tetramethylammonium)ethylene. The separation of Cr(III), present in the waste together with other metals/components, takes place during the electrolysis. The separation consists in that at the first stage Cr(III) on the anode is oxidized (at least partially) to soluble Cr(VI) compounds, and subsequently a selective membrane is used through which the Cr(VI) ions (anions) thus obtained are transmitted to another part of the electrolysis cell, where chromium in the form of Cr(VI) anion is collected, e.g. by way of precipitation of insoluble salts.

DE 639446 C discloses a process for electrowinning of chromium as a thick layer from an acidic electrolyte comprising chromium, using a lead anode and a cathode made of copper or iron, which is preferably at least 10 times smaller than the anode, wherein electrolysis is carried out at a constant cathode current density.

The essence of the invention is that the acidic electrolyte solution with a Cr(VI) ion concentration of more than 0.05 g/l is subjected to electrolysis using an anode made of steel or lead and a cathode made of steel, graphite or glassy carbon that is at least 10 times smaller than the anode, wherein the electrolysis is carried out potentiostatically or galvanostatically. For the lead anode, the cathode potential remains within the range from -2.9 V to -3.5 V and for the steel anode, the cathode potential remains within the range from -2.5 V to -3.0 V. The cathodic current density remains constant within the range from 0.06 A/cm² to 0.7 A/cm² in acidic solutions containing more than 50 g/l of chromium. Alternatively, the electrolysis is carried out using controlled pulsed current, wherein the cathodic current density remains constant within the range from 0.06 A/cm² to 0.7 A/cm² in acidic solutions containing more than 50 g/l of chromium, and the pulse off-time is from 10 to 20% of the electrolysis duration, which is over 10 s. The metallic chromium precipitates on the cathode in the form of flakes, powder or nanopowder.

Preferably, the electrolysis duration depends on the initial and final chromium content in the electrolyte, on the electrolyte volume, and on whether the metallic chromium obtained is supposed to be in the form of flakes, powder or nanopowder.

The main advantage of the above-presented invention is that it does not involve a very expensive stage of chemical reduction of Cr(VI) to Cr(III) ions, and the product obtained as a result of the method is metallic chromium, not its compound. Thus, the cost of the application of the solution in question is lower, and the product obtained, namely metallic chromium, is much more valuable than chromium salts, oxides or hydroxides obtained with prior art technology. It is particularly advantageous to use this invention for the selective waste electrolysis, since it enables the production of chromium in the form of flakes, powders and nanopowders with purity over 99.7%.

The invention is now described in more details by references to the following examples.

### Example I

In an electrochemical vessel thermostatted to 25°C there is a lead anode with an area of approx. 100 cm² which is also a reference electrode in a two-electrode system and the cathode is a graphite rod with an area of approx. 0.6 cm². The vessel is filled with electrolyte mainly composed of the following: 109.6 g/l Cr (mainly Cr(VI)), 10 g/l H₂SO₄ and 20.6 mg/l Cu.

The electrolysis is carried out potentiostatically with a potential of -3.5 V and an average current density of 0.385 A/cm² over 30 minutes.

### Example II

In an electrochemical vessel thermostatted to 25°C there is a lead anode with an area of approx. 100 cm² which is also a reference electrode in a two-electrode system and the cathode is a steel plate with an area of approx. 2.2 cm². The vessel is filled with electrolyte mainly composed of the following: 109.6 g/l Cr (mainly Cr(VI)), 10 g/l H₂SO₄ and 20.6 mg/l Cu.

The electrolysis is carried out galvanostatically with a potential of -3.28 V and current density of 0.227 A/cm² over 120 minutes.

### Example III

In an electrochemical vessel thermostatted to 25°C there is a lead anode with an area of approx. 100 cm² which is also a reference electrode in a two-electrode system and the cathode is a steel plate with an area of approx. 2 cm². The vessel is filled with electrolyte mainly composed of the following: 109.6 g/l Cr (mainly Cr(VI)), 10 g/l H₂SO₄ and 20.6 mg/l Cu.

The electrolysis is carried out using controlled pulsed current over the period of 3.5 hours with a 30 min break. Current density is 0.2 A/cm².

## Claims

1. A method for electrowinning of metallic chromium from acidic waste electrolytes **wherein** the acidic electrolyte solution with a Cr(VI) ion concentration of more than 0.05 g/l is subjected to electrolysis using an anode made of steel or lead and a cathode made of steel, graphite or glassy carbon that is at least 10 times smaller than the anode, wherein the electrolysis is carried out potentiostatically or galvanostatically, with the cathode potential for the lead anode remaining within the range from -2.9 V to -3.5 V and with the cathode potential for the steel anode remaining within the range from - 2.5 V to -3.0 V, while the cathodic current density remains constant within the range from 0.06 A/cm² to 0.7 A/cm² in acidic solutions containing more than 50 g/l of chromium, or using controlled pulsed current, wherein the cathodic current density remains constant within the range from 0.06 A/cm² to 0.7 A/cm² in acidic solutions containing more than 50 g/l of chromium, and the pulse off-time is from 10 to 20% of the electrolysis duration, which is over 10 s, while the metallic chromium precipitates on the cathode in the form of flakes, powder or nanopowder.

2. A method according to claim 1 **wherein** the electrolysis duration depends on the initial and final chromium content in the electrolyte, on the electrolyte volume, and on whether the metallic chromium obtained is supposed to be in the form of powder, flakes or nanopowder.

## Patentansprüche

1. Verfahren zur elektrolytischen Gewinnung von metallischem Chrom aus sauren Abfallelektrolyten, **wobei** die saure Elektrolytlösung mit einer Konzentration der Cr(VI)-Ionen von mehr als 0,05 g/l einer Elektrolyse mit Verwendung von eine Anode aus Stahl oder Blei und eine Kathode aus Stahl, Graphit oder Glaskohlenstoff, die mindestens zehnmal kleiner als Anode ist, wobei die Elektrolyse potentiostatisch oder galvanostatisch durchgeführt wird, wobei das Kathodenpotential für die Bleianode im Bereich von -2,9 V bis -3,5 V bleibt und das Kathodenpotential für die Stahlanode im Bereich von -2,5 V bis -3,0 V bleibt, während die kathodische Stromdichte im Bereich von 0,06 A/cm² bis 0,7 A/cm² in sauren Lösungen, die mehr als 50 g/l Chrom enthalten, konstant bleibt oder mit Verwendung eines gesteuerten gepulsten Stroms, wobei die kathodische Stromdichte im Bereich von 0,06 A/cm² bis 0,7 A/cm² in sauren Lösungen, die mehr als 50 g/l Chrom enthalten, konstant bleibt und die Ausschaltzeit des Pulses von 10 bis 20% der Elektrolysedauer beträgt, d.h. über 10 s, unterworfen wird, während das metallische Chrom in Form von Flocken, Pulver oder Nanopulver an der Kathode ausfällt.

2. Verfahren nach Anspruch 1, **wobei** die Elektrolysedauer vom anfänglichen und endgültigen Chromgehalt im Elektrolyten, vom Elektrolytvolumen und davon, ob das erhaltene metallische Chrom in Form von Pulver, Flocken oder Nanopulver vorliegen soll abhängt.

## Revendications

1. Une méthode d'électroextraction de chrome métallique à partir d'électrolytes de déchets acides, **dans laquelle** la solution électrolytique acide ayant une concentration en ions Cr (VI) supérieure à 0,05 g/l est soumise à une électrolyse à l'aide d'une anode en acier ou en plomb et d'une cathode en acier, en graphite ou en carbone vitreux qui est au moins 10 fois plus petite que l'anode, dans laquelle l'électrolyse est réalisée par voie potentiostatique ou galvanostatique, le potentiel cathodique de l'anode en plomb restant dans la plage de -2,9 V à -3,5 V et le potentiel cathodique de l'anode en acier restant dans la plage de -2,5 V à -3,0 V, tandis que la densité de courant cathodique reste constante dans la plage de 0,06 A/cm² à 0,7 A/cm² dans des solutions acides contenant plus de 50 g/l de chrome, ou en utilisant un courant pulsé contrôlé, dans laquelle la densité de courant cathodique reste constante dans la plage de 0,06 A/cm² à 0,7 A/cm² dans des solutions acides contenant plus de 50 g/l de chrome, et le temps de repos d'impulsion est de 10 à 20% de la durée de l'électrolyse, qui est plus de 10 secondes, tandis que le chrome métallique précipite sur la cathode sous forme de flocons, de poudre ou de nanopoudre.

2. Une méthode selon la revendication 1, **dans laquelle** la durée de l'électrolyse dépend de la teneur initiale et finale en chrome dans l'électrolyte, du volume de l'électrolyte et de la question si le chrome métallique obtenu est censé se présenter sous forme de poudre, de flocons ou de nanopoudre.
